

# UNITED STATES PATENT OFFICE.

LUDWIG MOND, OF NORTHWICH, COUNTY OF CHESTER, AND CARL LANGER,  
OF SOUTH HAMPSTEAD, COUNTY OF MIDDLESEX, ENGLAND.

## PROCESS OF OBTAINING HYDROGEN GAS.

### SPECIFICATION forming part of Letters Patent No. 417,068, dated December 10, 1889.

Application filed March 7, 1889. Serial No. 302,323. (No specimens.) Patented in England September 1, 1888, No. 12,608; in France February 28, 1889, No. 196,381; in Belgium February 28, 1889, No. 85,201, and in Italy March 31, 1889, XXIX, 25,043, XLIX, 150.

*To all whom it may concern:*

Be it known that we, LUDWIG MOND and CARL LANGER, subjects of the Queen of Great Britain, and residents of Northwich and South Hampstead, respectively, both in the Kingdom of England, have invented certain new and useful Improvements in the Process of Obtaining Hydrogen Gas, (which has been patented in England, No. 12,608, dated September 1, 1888; in France, No. 196,381, dated February 28, 1889; in Belgium, No. 85,201, dated February 28, 1889, and in Italy, XXIX, 25,043, XLIX, 150, dated March 31, 1889,) of which the following is a specification.

5 By the distillation or incomplete combustion, in presence or in the absence of steam, of oil, lignite, wood, coke, animal carbon, or organic substances in general, gases are obtained which consist, chiefly, of hydrogen, carburets 20 of hydrogen, monoxide and dioxide of carbon, and a greater or less quantity of nitrogen.

The object of our invention is to eliminate from these gases the monoxide of carbon and the carburets of hydrogen, and at the same 25 time to increase the amount of hydrogen contained.

If a mixture of monoxide of carbon or of carburet of hydrogen and steam be heated to white heat, the latter is decomposed and 30 the carbon of the gases is oxidized to a dioxide and the hydrogen set at liberty. The high temperature required for this reaction renders it of little profit, and it is difficult to produce it on an industrial scale.

35 We have found that if monoxide of carbon and hydrocarburets be placed in contact with nickel or metallic cobalt at a temperature not exceeding red heat these gases are decomposed into carbon and dioxide of carbon on the one hand and hydrogen on the other. The free carbon so formed placed in contact with steam at a moderate temperature decomposes the latter and forms dioxide of carbon and hydrogen. If the steam and 45 the gases are mixed from the commencement, the two reactions take place simultaneously, and the result is a gas practically free from monoxide of carbon and hydrocarburets. It

is quite possible to attain our object by carrying out consecutively the two above-mentioned reactions and by repeating them continually with the same quantity of nickel and cobalt, which will always be regenerated. We prefer, however, to carry out these two reactions simultaneously, at the same time employing the least possible amount of nickel and cobalt. With this object we spread the aforesaid metals on an indifferent refractory and porous material. For example, we saturate pieces of pumice-stone with a solution of chloride of nickel or cobalt, dry and reduce at a high temperature with hydrogen.

To carry out our invention, we lead the gases, with an excess of steam, into retorts or cylinders fixed in a suitable furnace and containing pieces of pumice-stone impregnated with nickel or cobalt, as above mentioned. If nickel be used, the reaction takes place at a temperature of 350° or 400° centigrade; if cobalt is used, at a temperature of 400° or 450° centigrade. The reactions which take place between the gas and the steam produce heat, so that the given temperature once reached the reaction goes on of itself, without need of external heating beyond the heat introduced by the hot gases. It may, however, be advantageous to use gases or steam, or both, heated to a suitable temperature before they are placed in the retorts. The gases so treated contain little or no monoxide of carbon.

To obtain pure hydrogen from the mixture of carbonic acid and hydrogen, the mixture is passed over or through layers of lime or of caustic alkali.

We claim as our invention—

1. The process of obtaining hydrogen from hydrogen contaminated with carbon monoxide or hydrocarbons, which consists in subjecting such contaminated hydrogen to the action of metallic nickel or cobalt and steam at the temperature described, and separating the carbon dioxide thereby formed by subjecting the resultant gases to the action of caustic lime or alkali.

2. The improvement in the process of ob-

50

55

60

65

70

75

80

85

95

taining hydrogen free from carbon monoxide or hydrocarbons, which consists in subjecting hydrogen contaminated with carbon monoxide or hydrocarbons to the action of metallic nickel or cobalt at the temperatures substantially as described.

3. The improvement in the process of obtaining hydrogen, which consists in subjecting the mass of nickel or cobalt and carbon (formed by subjecting gases containing carbon monoxide or hydrocarbons to the action of metallic nickel or cobalt at a suitable temperature) to the action of steam substantially at the temperature set forth, whereby a mixture of carbon dioxide and hydrogen is obtained.

4. The improvement in the process of obtaining hydrogen free from carbon monoxide or hydrocarbons, which consists in exposing hydrogen contaminated with carbon monoxide or hydrocarbons, or both, to the joint action of steam and of metallic nickel or cobalt at a temperature substantially as described.

In testimony whereof we have signed our names to this specification in the presence of two subscribing witnesses.

LUDWIG MOND,  
CARL LANGER.

Witnesses:

ALFRED J. BOULT,  
HARRY B. BRIDGE.